

Dec. 27, 1938.

H. T. LANG ET AL

2,141,307

COMMUTATOR

Filed Sept. 10, 1937

Fig.1.



Fig.2.



Inventors:

\*Henry T. Lang,  
Ralph E. Dunbar,

by *Henry E. Dunbar*  
Their Attorney.

## UNITED STATES PATENT OFFICE

2,141,307

## COMMUTATOR

Henry T. Lang, Cleveland, and Ralph E. Dunbar,  
East Cleveland, Ohio, assignors to Electric  
Vacuum Cleaner Company, Inc., Cleveland,  
Ohio, a corporation of New York

Application September 10, 1937, Serial No. 163,278

8 Claims. (Cl. 171—320)

The present invention relates to commutators for dynamo-electric machines.

It has been customary to insulate the copper segments of commutators with strips of mica arranged between the segments. Due to its mechanical strength and insulating properties, mica is a very satisfactory material. It is, however, much harder than the copper segments so that it has been necessary to undercut the mica by sawing slots between the adjacent segments of the commutator. The slotting or undercutting removes the mica adjacent the brush engaging surfaces and therefore permits the use of less abrasive soft carbon brushes. If the mica is not undercut very abrasive brushes must be used; otherwise the copper will be worn down faster than the mica and as a result the mica will project beyond the copper segments causing the brushes to jump which results in excessive sparking which burns the commutator. Even with undercutting, unless great pains are taken, some mica may be left in the slots and as soon as this mica is reached the brushes will be worn away very rapidly.

The object of our invention is to provide an improved construction and arrangement in commutators which will overcome some of the disadvantages of mica insulation, and for a consideration of what I believe to be novel and my invention, attention is directed to the accompanying description and the claims appended thereto.

In the accompanying drawing, Fig. 1 is a diagrammatic view of a commutator embodying my invention, and Fig. 2 is a fragmentary sectional view of the commutator.

Referring to the drawing, there is drawn a typical commutator having copper segments 1 insulated by strips of insulation material 2 clamped therebetween. As shown in Fig. 2 the ends of the segments are cut away to provide notches 3 for receiving clamping members 4. One of the clamping members is integral with a sleeve 5 on which is threaded a nut 6 for effecting the clamping action. Suitable insulation 7 is arranged between the segments and the clamping members and the sleeve. The sleeve may serve as a means for attaching the commutator to a shaft 8.

The segment insulation 2 is made of pressboard or other material having the properties of pressboard. Pressboard is paper which obtains its good mechanical properties such as denseness by "mechanical hydration" or "beating" followed by calendering which may be either "glaze rolling" or "super calendering". The term "mechanically

hydrated" is used to designate the process of manufacture in which the cellulose is hydrated in a paper beater as distinguished from chemical hydration by zinc chloride, sulphuric acid or other cellulose solvents such as used in the manufacture of vulcanized fiber. Chemically hydrated cellulose is not as satisfactory since it is chemically less stable under heat, which causes embrittlement, due to the degradation of the cellulose by the action of the cellulose solvent which breaks down the primary and secondary valence bonds of the cellulose. Due to the mechanical hydration and the subsequent compression, the cellulose fibers are intimately bonded together and held in a highly compressed condition producing a tough material having high compressive strength. Other materials which comprise cellulose fibers having the chemical stability of mechanically hydrated cellulose which are bonded together and held in a highly compressed condition are satisfactory for segment insulation. Glaze rolling is preferable to super calendering due to the smooth surface which more intimately contacts the sides of the segments and also to the fact that higher densities are obtained. The density of the pressboard is in the vicinity of 1.3 but is subject to considerable variation. The density of samples of different lots of the same grade of pressboard from the same manufacturer has been observed to vary from 1.13 to slightly above 1.5. All of these lots were used for segment insulation and proved satisfactory. It is obviously difficult to set a definite figure for the density of the pressboard. It is felt that the density is best described as "of the order of 1.3". Various grades of pressboard, being sold commercially, have been found satisfactory for segment insulation. Among these are 100% rag pressboards, sold under the trade-names of Armo, Duro, Spaldo, and Manning #300. These grades of pressboard are made in sheets and are glaze rolled. A similar material made in continuous strips is available under the trade-name of Vosite. Other pressboards made from mixtures of rag and wood pulp have been tried and found satisfactory. One example of this type of pressboard is sold under the trade-name of Tufelec which comprises a mixture of 75% rag and 25% kraft. This latter pressboard is super calendered instead of glaze-rolled. A glaze-rolled pressboard having 50% rag and the remainder of wood pulp has also been tried and found satisfactory. All of the pressboards mentioned above have the common characteristic of high compressive strength due to the high density and chemical stability under tempera-

tures usually encountered in commutators. This means that the commutator segments are firmly held in position so that the segments cannot move radially outward producing high bars which result in destructive sparking. In addition, the pressboards are less abrasive than copper and under normal "black" commutation wear substantially flush with the copper. This eliminates the need for undercutting. There may be some 10 pitting of the brush engaging surfaces of the segment insulation due to sparking. A further advantage of the pressboard insulation is that the particles which are worn away during the operation of the commutator are not abrasive and consequently the wear on the commutator segments is greatly decreased. The pressboard should be free from acid and preferably alkaline since the presence of acid greatly decreases the resistance to heat.

20 What we claim as new and desire to secure by Letters Patent of the United States is:

1. A commutator having segments held in spaced relation and insulated from each other by pressboard made from mechanically hydrated stock and having a density of the order of 1.3.
2. A commutator having segments held in spaced relation and insulated from each other by glaze-rolled pressboard having the properties of a pressboard made from mechanically hydrated paper stock.
3. A commutator having segments held in spaced relation and insulated from each other by

glaze-rolled pressboard having the properties of pressboard made from a mixture of mechanically hydrated rag stock and wood pulp.

4. A commutator having segments held in spaced relation and insulated from each other by a mechanically hydrated rag stock pressboard having a density of the order of 1.3.

5. A commutator having segments held in spaced relation and insulated from each other by pressboard made from cellulose having the properties of mechanically hydrated cellulose.

6. A commutator having segments held in spaced relation and insulated from each other by fibrous insulation comprising cellulose fibers having the properties of mechanically hydrated cellulose which are intimately bonded together and held in a highly compressed condition.

7. A commutator having segments held in spaced relation and insulated from each other by a super calendered mechanically hydrated cellulose pressboard having a density of the order of 1.3.

8. A commutator having segments held in spaced relation and insulated from each other by fibrous insulation comprising cellulose fibers having the properties of mechanically hydrated cellulose which are intimately bonded together and held in a highly compressed condition, said insulation having a density of the order of 1.3.

30

HENRY T. LANG.  
RALPH E. DUNBAR.